

# UNITED STATES PATENT OFFICE.

JOHN N. PRING, OF NEW YORK, N. Y., ASSIGNOR TO ELMER A. SPERRY, OF BROOKLYN, NEW YORK.

## ELECTROLYTIC PROCESS FOR REFINING NICKEL.

No. 874,864.

Specification of Letters Patent.

Patented Dec. 24, 1907.

Application filed November 8, 1906. Serial No. 342,491.

*To all whom it may concern:*

Be it known that I, JOHN N. PRING, a subject of Great Britain, residing at New York, in the county of New York and State of New York, have invented new and useful Improvements in Electrolytic Processes for Refining Nickel, of which the following is a specification.

My invention relates to the purification of nickel and it consists more particularly in first dissolving the crude nickel together with the associated metals for instance as sulfates or, beginning with one of the salts especially such as is obtained in refining copper or other metals and which may contain such impurities as zinc, iron, cobalt and copper. Beside these metals it is possible to free the nickel or the nickel and cobalt from such substances as As. Sb. Bi. Pb. and Hg.

20 To illustrate one method of carrying out the process I will describe the case of separation of nickel from copper refining waste in the form of crude sulfate. This is first dissolved in water to which is added a little suitable sulfid, such for instance as Na<sub>2</sub>S or for instance a little nickel sulfid freshly precipitated and which may be taken from the process later on. During this treatment it is well to agitate the solution which is then 25 filtered or the solution may be filtered over a small amount of the nickel sulfid. Copper is thus thrown out as the sulfid, together with the second series of metals recited above. The filtrate is then digested with any soluble 30 sulfid such as an alkaline sulfid for instance, with black ash or calcium sulfid which convert and precipitate as sulfids the following metals: Ni. Co. Fe. Zn. and Mn. I now proceed without separating the sulfids, to digest

35 the agitated liquor with a suitable acid to the point of neutralization. I now add an excess of an acid which I have discovered will redissolve the above named foreign sulfids except cobalt and including manganese 40 only: hydrochloric acid is an example of such a solvent; I now agitate for a short period whereupon it is found that nickel sulfid and cobalt sulfid alone remain undissolved or I may proceed to separate the solids, wash 45 and treat in dilute solvent for the metals other than Ni. and Co. as sulfids. These will readily settle, whereupon by decantation and suitable washing, either with or without

filtering, the sulfids are found to be unassociated with the other metals and are particularly pure. For some purposes these may be considered to be the commercial products of the process or they can then be treated by any of the well known processes for separation of nickel and cobalt or we may proceed either with or without such separation as follows to reduce to the metallic state. This step may be conducted in any form of reduction furnace or by roasting or it may be electrolytic in its nature and in such case is based upon the fact that nickel sulfid is converted into nickel chlorid by Cl<sub>2</sub> on heating, or as I have discovered by nascent chlorin as generated at the anode or in the anode compartment of an electrolytic cell, electrolyzing a chlorid. This cell may contain a nickel or other suitable cathode which receives the deposit of nickel. The electrolyte may consist of a solution of nickel chlorid, the anodes being plain graphite plates contained within a suitable diaphragm porous cell, or porous partition. The nickel sulfid is fed into the anolyte and is held there, more or less in a state of suspension, or may be fed in a thin layer down the flat faces of the anode. During electrolysis nickel is deposited on the cathode in a fine coherent form and practically no chlorin is evolved from the anode compartment. The Ni<sub>2</sub> is converted into nickel chlorid (NiCl<sub>2</sub>) and sulfur is found to gradually accumulate in the anode chamber; this is periodically or otherwise removed and separated from the sulfid in any suitable manner as for instance, by sublimation, the sulfids being returned to the process and the sulfur condensed and recovered as the flowers of sulfur or in other suitable form.

I do not care to limit myself to the exact process stated above which is simply used to illustrate one method of carrying out my invention for instance solution other than the sulfate may be employed as will readily be understood; also some of the steps may be varied and where the impurity will permit it is obvious that same may be omitted without interfering with the scope of the invention as stated in the claims hereto annexed and forming a part hereof and the invention extends to such use. It will also be readily understood that a sulphydrate may be employed in lieu of the sulfid mentioned above.

I claim:

1. The method of refining impure or crude nickel which consists in treating it in a suitable solution with a soluble sulfid, 5 treating the liquid which bears the resulting solids with a solvent for the foreign bodies, separating the remaining solids and electrolyzing them.
2. The method of refining impure or 10 crude nickel which consists in treating it in a suitable solution with a soluble sulfid, treating the liquid which bears the resulting solids with a solvent for the foreign bodies, separating the remaining solids and electrolyzing them in the presence of a chlorid.
3. The method of refining impure or 15 crude nickel which consists in treating it in a suitable solution with a soluble sulfid, treating the liquid which bears resulting 20 solids with a solvent for the foreign bodies,

separating the remaining solids and electrolyzing them in a compartment cell and in the anode compartment of such cell.

4. The method of refining impure or 25 crude nickel which consists in treating it in a suitable solution with a soluble sulfid, treating the liquid which bears the resulting solids with a solvent for the foreign bodies, separating the remaining solids and electrolyzing them in an electrolytic cell in contact with an inert anode and depositing nickel at the cathode.

In testimony whereof I have hereunto set my hand in presence of two subscribing witnesses.

JOHN N. PRING.

Witnesses:

THOMAS ROBINSON,  
E. A. SPERRY.